

H. R. SWARTLEY, JR.

ANODE.

APPLICATION FILED FEB. 25, 1916.

**1,263,959.**

Patented Apr. 23, 1918.



INVENTOR

*H. R. Swartley, Jr.*  
BY

*J. B. Hendley*

ATTORNEY

# UNITED STATES PATENT OFFICE.

HENRY R. SWARTLEY, JR., OF MANHASSET, NEW YORK, ASSIGNOR TO DAVIS-BOURNONVILLE COMPANY, OF JERSEY CITY, NEW JERSEY, A CORPORATION OF NEW YORK.

## ANODE.

1,263,959.

Specification of Letters Patent. Patented Apr. 23, 1918.

Application filed February 25, 1916. Serial No. 80,414.

*To all whom it may concern:*

Be it known that I, HENRY R. SWARTLEY, Jr., a citizen of the United States, and a resident of Manhasset, Long Island, in the 5 county of Nassau and State of New York, have invented certain new and useful Improvements in Anodes, of which the following is a specification.

The invention is an improved anode for 10 water electrolyzers. It is customary to make these electrodes of iron, and in order to protect them from oxidation by the oxygen liberated at their surfaces the general 15 practice is to plate them with nickel. Instead of the electro-deposited surfaces here- tofore employed, I propose to provide these anodes with sprayed metal surfaces, that is to say, coatings composed of fine nickel par- ticles rendered molten and impacted on the 20 iron by means of a blast. Metal coatings

of this nature are known, but have not heretofore been applied to anodes, for which such a coating possesses a peculiar advantage. This advantage is the special rough or uneven surface, due to the character of the 25 coating, the structure of which is necessarily different from one formed electrolytically, the effect of such surface being to promote the liberation of the oxygen. It will be understood that the shape of the 30 anode, or whether the electrode is uni-polar or bi-polar, is not material.

The drawing shows an illustrative form of electrode and indicates the sprayed nickel surface. 35

What I claim as new is:

An anode having a permanent continuous surface of sprayed nickel.

HENRY R. SWARTLEY, JR.